

## UNITED STATES PATENT OFFICE

1,921,417

## ALLOY

Robert H. Leach, Fairfield, Conn., assignor to  
 Handy & Harman, New York, N. Y., a Corporation of New York

No Drawing. Application May 23, 1933  
 Serial No. 672,469

## 4 Claims. (Cl. 75—1)

This invention relates to alloys used for brazing and welding purposes and is concerned more particularly with a novel quaternary alloy which has relatively low melting and flow points and can 5 be used with great facility for the production of joints of excellent tensile strength, as, for example, between objects of copper and brass.

The new alloy consists of silver ranging from about 5% to about 20%, zinc from about 5% to 10 about 25%, copper from about 55% to about 80%, and phosphorus from about 2% to about 5%. Typical examples of the new alloy may have approximately the following percentages:

|            | Per cent |
|------------|----------|
| 1. Silver  | 5        |
| Copper     | 65       |
| Zinc       | 25       |
| Phosphorus | 5        |
| 2. Silver  | 10       |
| Copper     | 60       |
| Zinc       | 25       |
| Phosphorus | 5        |
| 3. Silver  | 20       |
| Copper     | 55       |
| Zinc       | 20       |
| Phosphorus | 5        |

These and other alloys within the ranges mentioned offer the advantages of having melting points which are substantially lower than those of the alloys commonly known as "silver solders" and the new alloys have such physical properties that they can be hot worked into forms which are convenient for use. When the new alloys are used in uniting objects of copper, it is found that strong ductile joints can be made without flux.

The alloys within the ranges mentioned have 40 closely similar melting points, as, for instance, the alloy given in Example No. 1 has a melting point

of 1190° F. and the alloy of Example No. 3 has a melting point of 1130° F. The thermal properties of the new alloys permit their use in the uniting of objects at lower temperatures than are possible with similar alloys heretofore used for the 60 purpose and the physical properties of the new alloys and of the joints made therefrom are highly satisfactory for many uses. While the joints produced with the new alloys are not as strong as those produced by means of the alloy 65 of silver, copper and phosphorus disclosed in my Patent No. 1,829,903, issued November 3, 1931, the new alloys may be produced in forms having somewhat lower melting points than the patented alloy, and the joints have strength and 70 ductility which are entirely sufficient for a wide range of uses.

## What I claim is:

1. An alloy which consists of silver ranging from about 5% to about 20%, copper ranging 75 from about 55% to about 80%, zinc ranging from about 5% to about 25%, and phosphorus ranging from about 2% to about 5%.
2. An alloy which consists of silver ranging 80 from about 5% to about 10%, copper ranging from about 60% to about 80%, zinc ranging from about 5% to about 25%, and phosphorus ranging from about 2% to about 5%.
3. An alloy which consists of silver ranging 85 from about 10% to about 15%, copper ranging from about 60% to about 80%, zinc ranging from about 5% to about 25%, and phosphorus ranging from about 3% to about 5%.
4. An alloy which consists of silver ranging 90 from about 15% to about 20%, copper ranging from about 55% to about 75%, zinc ranging from about 5% to about 22%, and phosphorus ranging from about 3% to about 5%.

ROBERT H. LEACH. 95